

O. C. DURYEA AND M. C. WHITE:

ART OF BRIQUETING.

APPLICATION FILED FEB. 14, 1917.

1,371,671.

Patented Mar. 15, 1921.

*Fig. 1.*



*Fig. 2.*



Inventor

and Otto C. Duryea  
Morris C. White

Witness

Conrad W. Crocker

By Dryerforth Lee Chittenden

Attorney

# UNITED STATES PATENT OFFICE.

OTHO CROMWELL DURYEA, OF WATERBURY, CONNECTICUT, AND MORRIS COLUMBUS WHITE, OF OAKLAND, CALIFORNIA, ASSIGNEES TO AMERICAN BRIQUET MACHINE COMPANY, OF CHICAGO, ILLINOIS, A CORPORATION OF SOUTH DAKOTA.

## ART OF BRIQUETING.

1,371,671.

Specification of Letters Patent. Patented Mar. 15, 1921.

Application filed February 14, 1917. Serial No. 148,531.

*To all whom it may concern:*

Be it known that we, OTHO CROMWELL DURYEA and MORRIS COLUMBUS WHITE, citizens of the United States of America, respectively residing at Waterbury, New Haven county, Connecticut, and Oakland, Alameda county, California, have invented certain new and useful Improvements in the Art of Briquetting, of which the following is a specification.

Our invention relates to the uniting into an integral mass of a quantity of smaller particles of material and it consists in a method of accomplishing the result sought and in the product of that method.

For a long time it has been considered desirable to join a large number of particles of matter so as to form blocks, briquets or other masses of various forms and sizes, because comminuted matter thus joined into larger units and made more compact, could be more easily and economically handled and could be used in ways not possible with the material in smaller divisions.

The methods usually employed involve the use of pressure to compact the mass and generally some sort of binder to hold the particles together, but such joinder is not entirely satisfactory for the reason that the product is likely to disintegrate upon the application of a comparatively low heat and oftentimes by mere shock, such as that occasioned by the falling of the mass a short distance.

To meet the desire for a substantially solidified mass, we have devised the novel method about to be described, which consists in assembling a quantity of the smaller fragments or particles of material to be treated, applying pressure to force them closely together and then suddenly raising the pressure to a high degree.

The sudden and practically explosive application of increased pressure causes the individual fragments or particles to slide one upon another and the friction thus occasioned creates an intense heat at the proximate surfaces of the fragments and thereby fuses, welds or coheres those fragments into one mass, no longer a quantity of fragments closely associated, but a new product integral and substantially solid, suitable for an infinite variety of uses. The heat produced at the surfaces of union of the par-

ticles is distributed by conduction, and causes no appreciable rise in temperature of the mass. The explosive pressure applied, which may be maintained for an appreciable period of time, is above the elastic limit of the material treated.

This method may be practised in a variety of ways and with a variety of apparatus, but the one we have found most satisfactory is a press in which the fragments may be confined, brought into intimate contact and then be united by a sudden raising of the pressure, for instance by firing a charge of explosive mixture or by the sudden release of a confined fluid pressure behind the head or plunger in contact with the material to be treated.

Such a mechanical movement is shown and described in reissued Letters-Patent No. 12,957 issued May 18, 1909, the process in its present application is illustrated by the accompanying drawings, in which Figures 1 and 2 show successive stages of the operation of the process.

When thus practised, we have constructed a die, the male member 5 of which is attached to or formed by the plunger of the press. The matter to be treated, for instance iron borings or other comminuted or fragmentary matter 6 is fed into the cylinder part 7 of the die, which acts to confine it and prevents its escape from the pressure. The plunger is then entered into the die cylinder and forced therein sufficiently to bring the fragments into intimate contact as indicated in Fig. 1, this step in the process being comparatively slow. When this stage has been reached, the explosive charge in the press cylinder is fired and the force of the explosion drives the plunger farther into the die cylinder with tremendous power as indicated in Fig. 2, the blow resulting in that solidification which is the result we seek.

The tremendous pressure thus explosively applied may be relieved at once or held for an instant as may be found to best accommodate the particular material under treatment.

The mass of fragments, if of iron borings, will be found to have been united into a solid block which may be handled and used as that much pig iron might be used, constituting in itself a new and useful product,

and fragments of other substances may be solidified by the same method.

We do not limit ourselves to specific pressures as they will vary according to the material used, the size of the charges and the purposes for which the products are to be used, but we have found that in treating iron borings, in charges of three pounds, in a die of three inches diameter, a pressure 10 rising gradually to 10,000 pounds per square inch of surface of the die, followed by an explosive pressure of 130,000 pounds per square inch of upper surface of die produces very satisfactory results.

15 Nor do we limit ourselves to exploding gas as the means of securing the sudden raising of pressure. We may use some other expansive fluid—such as steam or compressed air—by retarding expansion and 20 providing means for sudden release, as it is very apparent that this would give the blow necessary to cause the desired result, but we prefer to use the explosive means described on account of the more direct application of 25 power in that way and the consequent saving in cost.

What we claim and desire to secure by Letters-Patent, is:—

1. As a new article of manufacture, a 30 block formed of small metallic fragments which have been welded into an approximately solid mass by applying a comparatively mild pressure and then the pressure suddenly raised to a high degree by explosive force by which the parts are practically welded together.

2. The process of forming into one mass a multiplicity of small metallic fragments which consists in confining the small frag-

ments, applying a mild pressure to bring 40 the fragments into intimate contact and then raising the pressure with great suddenness to a high degree to cause the fragments to be welded together.

3. The process of forming into one mass a 45 multiplicity of small metallic fragments which consists in confining the small fragments, applying comparatively mild pressure to bring the fragments into intimate contact with each other, then raising the 50 pressure with explosive suddenness and maintaining the high pressure for an appreciable interval to cause said fragments to be welded together into a substantially solid mass and then set in that form. 55

4. The process of forming into one mass a multiplicity of small metallic fragments, which consists in confining the small particles, applying a mild pressure and then raising the pressure with great suddenness to a 60 high degree, whereby said fragments are caused to slide one upon another and create a high degree of surface heat without materially raising the temperature of the mass as a whole. 65

5. The process of agglomerating smaller metallic masses, which consists in assembling them in a confined space, applying comparatively mild pressure, raising the pressure with explosive suddenness to a high 70 degree and maintaining a pressure beyond the elastic limit of the material for an appreciable time.

In testimony whereof, we have signed our names to this specification, this twentieth 75 day of November, 1916.

OTHO CROMWELL DURYEA.  
MORRIS COLUMBUS WHITE.